



US008774696B2

(12) **United States Patent**  
**Liu et al.**

(10) **Patent No.:** **US 8,774,696 B2**  
(45) **Date of Patent:** **Jul. 8, 2014**

(54) **DELIVERY APPARATUS**

(75) Inventors: **Yu Liu**, Mississauga (CA); **Sarah J. Vella**, Milton (CA); **Vladislav Skorokhod**, Concord (CA); **Gaetano J. Lavigne**, Burlington (CA); **Nan-Xing Hu**, Oakville (CA); **Gregory M. McGuire**, Oakville (CA)

(73) Assignee: **Xerox Corporation**, Norwalk, CT (US)

(\*) Notice: Subject to any disclaimer, the term of this patent is extended or adjusted under 35 U.S.C. 154(b) by 142 days.

(21) Appl. No.: **13/437,472**

(22) Filed: **Apr. 2, 2012**

(65) **Prior Publication Data**

US 2013/0259551 A1 Oct. 3, 2013

(51) **Int. Cl.**

**G03G 21/00** (2006.01)

(52) **U.S. Cl.**

USPC ..... **399/346**

(58) **Field of Classification Search**

USPC ..... 399/110, 176, 346  
See application file for complete search history.

(56) **References Cited**

## U.S. PATENT DOCUMENTS

|             |         |                   |
|-------------|---------|-------------------|
| 3,121,006 A | 2/1964  | Middleton et al.  |
| 4,387,980 A | 6/1983  | Ueno et al.       |
| 4,435,074 A | 3/1984  | Midorikawa et al. |
| 4,464,450 A | 8/1984  | Teuscher          |
| 4,587,189 A | 5/1986  | Hor et al.        |
| 4,664,995 A | 5/1987  | Horgan et al.     |
| 4,921,773 A | 5/1990  | Melnik et al.     |
| 5,069,993 A | 12/1991 | Robinette et al.  |

|                 |         |                                |
|-----------------|---------|--------------------------------|
| 5,384,929 A     | 1/1995  | Smith                          |
| 5,499,089 A     | 3/1996  | Tsukamoto et al.               |
| 5,646,718 A     | 7/1997  | Suwa et al.                    |
| 5,756,245 A     | 5/1998  | Esteghamatian et al.           |
| 6,434,357 B1    | 8/2002  | Maul et al.                    |
| 6,582,222 B1    | 6/2003  | Chen et al.                    |
| 6,869,918 B2    | 3/2005  | Cornelius                      |
| 7,428,402 B2    | 9/2008  | Hays et al.                    |
| 7,526,243 B2    | 4/2009  | Zaman et al.                   |
| 7,580,655 B2    | 8/2009  | Nukada et al.                  |
| 7,725,069 B2    | 5/2010  | Kawahara et al.                |
| 7,734,242 B2 *  | 6/2010  | Hatakeyama et al. .... 399/346 |
| 7,877,054 B1    | 1/2011  | Thayer et al.                  |
| 7,881,651 B2    | 2/2011  | Watanabe                       |
| 7,960,082 B2    | 6/2011  | Aziz et al.                    |
| 8,600,281 B2    | 12/2013 | Hu et al.                      |
| 2003/0049555 A1 | 3/2003  | Sakon et al.                   |
| 2003/0118372 A1 | 6/2003  | Kitano et al.                  |
| 2005/0163527 A1 | 7/2005  | Tombs                          |
| 2009/0087213 A1 | 4/2009  | Takaya et al.                  |

(Continued)

## FOREIGN PATENT DOCUMENTS

JP 2002357983 A \* 12/2002 ..... G03G 21/00

## OTHER PUBLICATIONS

Machine translation of JP 2002-357983.\*

(Continued)

*Primary Examiner* — Walter L Lindsay, Jr.

*Assistant Examiner* — Barnabas Fekete

(74) *Attorney, Agent, or Firm* — Hoffman Warnick LLC

(57) **ABSTRACT**

There is described an applicator for use in an image forming apparatus. The applicator comprises a blade applicator comprising an elastomeric matrix and a functional material dispersed therein. The applicator blade is positioned in a trailing position with respect to a surface and wherein the functional material diffuses from the elastomeric matrix to the surface.

**18 Claims, 6 Drawing Sheets**



(56)

**References Cited**

U.S. PATENT DOCUMENTS

2009/0162092 A1 6/2009 Hoshio  
2009/0185821 A1 7/2009 Iwamoto et al.  
2009/0220876 A1 9/2009 De Jong et al.  
2010/0189461 A1 7/2010 Shintani et al.  
2011/0033798 A1 2/2011 Kim et al.  
2011/0206430 A1 8/2011 Arai et al.

OTHER PUBLICATIONS

Walsh, U.S. Appl. No. 13/279,981, Office Action dated Nov. 6, 2013, 20 pages.

U.S. Appl. No. 13/192,252, filed Jul. 27, 2011.  
U.S. Appl. No. 13/192,215, filed Jul. 27, 2011.

U.S. Appl. No. 13/020,738, filed Feb. 3, 2011.  
U.S. Appl. No. 12/845,662, filed Jul. 28, 2010.  
U.S. Appl. No. 13/286,905, filed Nov. 1, 2011.  
U.S. Appl. No. 13/279,981, filed Oct. 24, 2011.  
U.S. Appl. No. 13/320,414, filed Dec. 15, 2011.  
U.S. Appl. No. 13/354,022, filed Jan. 19, 2012.  
U.S. Appl. No. 13/426,836, filed Mar. 22, 2012.  
Sanghera, U.S. Appl. No. 13/354,022, Office Action dated Aug. 8, 2013, 25 pages.  
U.S. Appl. No. 13/533,475, Notice of Allowance and Fees Due, Dec. 9, 2013, 20 pages.  
U.S. Appl. No. 13/426,836, Ex Parte Quayle Action dated Mar. 20, 2014, 18 pages.  
U.S. Appl. No. 13/326,414, Office Action, Mar. 28, 2014, 19 pages.

\* cited by examiner



FIG. 1



FIG. 2



FIG. 3



FIG. 4



**FIG. 5**



**FIG. 6**



**FIG. 7**



FIG. 8



FIG. 9



FIG. 10

**1**  
**DELIVERY APPARATUS**

FIELD OF USE

This disclosure is generally directed to the delivery of a functional material or lubricant to the surface of imaging members, photoreceptors, photoconductors, and the like.

BACKGROUND

In electrophotography or electrophotographic printing, the charge retentive surface, typically known as a photoreceptor, is electrostatically charged, and then exposed to a light pattern of an original image to selectively discharge the surface in accordance therewith. The resulting pattern of charged and discharged areas on the photoreceptor form an electrostatic charge pattern, known as a latent image, conforming to the original image. The latent image is developed by contacting it with a finely divided electrostatically attractable powder known as toner. Toner is held on the image areas by the electrostatic charge on the photoreceptor surface. Thus, a toner image is produced in conformity with a light image of the original being reproduced or printed. The toner image may then be transferred to a substrate or support member (e.g., paper) directly or through the use of an intermediate transfer member, and the image affixed thereto to form a permanent record of the image to be reproduced or printed. Subsequent to development, excess toner left on the charge retentive surface is cleaned from the surface. The process is useful for light lens copying from an original or printing electronically generated or stored originals such as with a raster output scanner (ROS), where a charged surface may be imagewise discharged in a variety of ways.

The described electrophotographic copying process is well known and is commonly used for light lens copying of an original document. Analogous processes also exist in other electrophotographic printing applications such as, for example, digital laser printing and reproduction where charge is deposited on a charge retentive surface in response to electronically generated or stored images.

To charge the surface of a photoreceptor, a contact type charging device has been used, such as disclosed in U.S. Pat. No. 4,387,980 and U.S. Pat. No. 7,580,655, which are incorporated herein by reference in their entirety. The contact type charging device, also termed “bias charge roll” (BCR), includes a conductive member which is supplied a voltage from a power source with a D.C. voltage superimposed with an A.C. voltage of no less than twice the level of the D.C. voltage. The charging device contacts the image bearing member (photoreceptor) surface, which is a member to be charged.

Electrophotographic photoreceptors can be provided in a number of forms. For example, the photoreceptors can be a homogeneous layer of a single material, such as vitreous selenium, or it can be a composite layer containing a photoconductive layer and another material. In addition, the photoreceptor can be layered. Multilayered photoreceptors or imaging members have at least two layers, and may include a substrate, a conductive layer, an optional undercoat layer (sometimes referred to as a “charge blocking layer” or “hole blocking layer”), an optional adhesive layer, a photogenerating layer (sometimes referred to as a “charge generation layer,” “charge generating layer,” or “charge generator layer”), a charge transport layer, and an optional overcoating layer in either a flexible belt form or a rigid drum configuration. In the multilayer configuration, the active layers of the photoreceptor are the charge generation layer (CGL) and the

charge transport layer (CTL). Enhancement of charge transport across these layers provides better photoreceptor performance. Multilayered flexible photoreceptor members may include an anti-curl layer on the backside of the substrate, opposite to the side of the electrically active layers, to render the desired photoreceptor flatness.

In recent years, organic photoreceptors have been widely used for electrographic purposes. This is because organic photoreceptors are easy to prepare at low cost and have the advantages of mechanical flexibility, easy disposability and environmental sustainability. However, the microcorona generated during repetitive charging, damages the organic photoconductor, resulting in a rapid wear of the imaging surface and shortening the life of the photoreceptor.

To further increase the service life of the photoreceptor, use of overcoat layers has also been implemented to protect photoreceptors and improve performance, such as wear resistance. However, these low wear overcoats are associated with poor image quality due to A-zone deletion in a humid environment as the wear rates decrease to a certain level. In addition, high friction associated with low wear overcoats in A-zone also causes severe issues with BCR charging systems, such as motor failure due to high friction/torque and blade damage. As a result, use of a low wear overcoat with BCR charging systems is still a challenge, and there is a need to find ways to increase the life of the photoreceptor with excellent image quality and charging performance.

SUMMARY

Disclosed herein is an applicator for use in an image forming apparatus. The applicator comprises a blade applicator comprising an elastomeric matrix and a functional material dispersed therein. The applicator blade is positioned in a trailing position with respect to a surface and wherein the functional material diffuses from the elastomeric matrix to the surface.

Disclosed herein is an image forming apparatus that includes an imaging member having a charge retentive surface for developing an electrostatic latent image thereon. The imaging member comprises a substrate and a photoconductive member disposed on the substrate. The image forming apparatus includes a charging unit for applying an electrostatic charge on the imaging member to a predetermined electric potential. The image forming apparatus includes an applicator disposed in contact with the surface of the imaging member or a surface of the charging unit, wherein the applicator comprises a blade applicator comprising an elastomeric matrix and a functional material dispersed therein, wherein the applicator blade is positioned in contact and in a trailing position with respect to the surface of the imaging member or a surface of the charging unit.

Disclosed herein is an applicator for use in an image forming apparatus. The applicator comprises a blade applicator comprising a first layer comprising an elastomeric matrix and a functional material dispersed therein, and a second layer comprising an elastomer disposed on the first layer, wherein the second layer is positioned in a trailing position with respect to a surface and wherein the functional material diffuses through the second layer to the surface.

BRIEF DESCRIPTION OF THE DRAWINGS

The accompanying drawings, which are incorporated in and constitute a part of this specification, illustrate several

embodiments of the present teachings and together with the description, serve to explain the principles of the present teachings.

FIG. 1 is a cross-sectional view of an imaging member in a drum configuration according to the present embodiments.

FIG. 2 is a cross-sectional view of an imaging member in a belt configuration according to the present embodiments.

FIG. 3 is a cross-sectional view of a system implementing a blade applicator according to the present embodiments.

FIG. 4 is an alternative cross-sectional view of a system implementing a blade applicator according to the present embodiments.

FIG. 5 is an alternative cross-sectional view of a system implementing a blade applicator according to the present embodiments.

FIG. 6 is a side view of a blade applicator according to the present embodiments.

FIG. 7 is a side view of a blade applicator according to the present embodiments.

FIG. 8 is a side view of a blade applicator according to the present embodiments.

FIG. 9 is a side view with various embodiments of the tip of the of a blade applicator.

FIG. 10 is a print test demonstrating A-zone deletion results of prints made with the system according to embodiments described herein.

It should be noted that some details of the figures have been simplified and are drawn to facilitate understanding of the embodiments rather than to maintain strict structural accuracy, detail, and scale.

#### DESCRIPTION OF THE EMBODIMENTS

In the following description, reference is made to the chemical formulas that form a part thereof, and in which is shown by way of illustration specific exemplary embodiments in which the present teachings may be practiced. These embodiments are described in sufficient detail to enable those skilled in the art to practice the present teachings and it is to be understood that other embodiments may be utilized and that changes may be made without departing from the scope of the present teachings. The following description is, therefore, merely exemplary.

Notwithstanding that the numerical ranges and parameters setting forth the broad scope of the disclosure are approximations, the numerical values set forth in the specific examples are reported as precisely as possible. Any numerical value, however, inherently contains certain errors necessarily resulting from the standard deviation found in their respective testing measurements. Moreover, all ranges disclosed herein are to be understood to encompass any and all sub-ranges subsumed therein. For example, a range of "less than 10" can include any and all sub-ranges between (and including) the minimum value of zero and the maximum value of 10, that is, any and all sub-ranges having a minimum value of equal to or greater than zero and a maximum value of equal to or less than 10, e.g., 1 to 5. In certain cases, the numerical values as stated for the parameter can take on negative values. In this case, the example value of range stated as "less than 10" can assume negative values, e.g. -1, -2, -3, -10, -20, -30, etc.

The disclosed embodiments are directed generally to a delivery applicator for applying a layer of a functional material that acts as a lubricant on an imaging member surface. The layer of functional material acts as a barrier against moisture and/or surface contaminants, thereby protecting the surface of the imaging member. The application of the lubricant provides improved wear resistance, low friction, and

reduced image defects due to deletion in high humidity conditions, which leads to improved xerographic performance in imaging members.

A long life photoreceptor (P/R) enables significant cost reduction. Generally P/R life extension is achieved with a wear-resistant overcoat. However, wear resistant overcoats are associated with an increase in A-zone deletion (a printing defect that occurs at high humidity). Most organic photoreceptor materials require a minimal wear rate of 2 nm/Kcycle (Scorotron charging system) or from about 5 nm/Kcycle to about 10 nm/Kcycle (BCR charging system) in order to suppress A-zone deletion. In addition, wear-resistant overcoats cause a higher friction/torque that results in issues with BCR charging systems, such as motor failure and blade damage at the earlier stage of printing, which results in streaking of toner in prints.

FIG. 1 is an exemplary embodiment of a multilayered electrophotographic imaging member or photoreceptor having a drum configuration. The substrate may further be in a cylinder configuration. As can be seen, the exemplary imaging member includes a rigid support substrate 10, an electrically conductive ground plane 12, an undercoat layer 14, a charge generation layer 18 and a charge transport layer 20. An optional overcoat layer 32 disposed on the charge transport layer 20 may also be included. The substrate 10 may be a material selected from the group consisting of a metal, metal alloy, aluminum, zirconium, niobium, tantalum, vanadium, hafnium, titanium, nickel, stainless steel, chromium, tungsten, molybdenum, and mixtures thereof. The substrate 10 may also comprise a material selected from the group consisting of a metal, a polymer, a glass, a ceramic, and wood.

The charge generation layer 18 and the charge transport layer 20 form an imaging layer described herein as two separate layers. In an alternative to what is shown in the figure, the charge generation layer 18 may also be disposed on top of the charge transport layer 20. It will be appreciated that the functional components of these layers may alternatively be combined into a single layer.

FIG. 2 shows an imaging member or photoreceptor having a belt configuration according to the embodiments. As shown, the belt configuration is provided with an anti-curl back coating 1, a supporting substrate 10, an electrically conductive ground plane 12, an undercoat layer 14, an adhesive layer 16, a charge generation layer 18, and a charge transport layer 20. An optional overcoat layer 32 and ground strip 19 may also be included. An exemplary photoreceptor having a belt configuration is disclosed in U.S. Pat. No. 5,069,993, which is hereby incorporated by reference in its entirety.

As discussed above, an electrophotographic imaging member generally comprises at least a substrate layer, an imaging layer disposed on the substrate and an optional overcoat layer disposed on the imaging layer. In further embodiments, the imaging layer comprises a charge generation layer disposed on the substrate and the charge transport layer disposed on the charge generation layer. In other embodiments, an undercoat layer may be included and is generally located between the substrate and the imaging layer, although additional layers may be present and located between these layers. The imaging member may also include an anti-curl back coating layer in certain embodiments. The imaging member can be employed in the imaging process of electrophotography, where the surface of an electrophotographic plate, drum, belt or the like (imaging member or photoreceptor) containing a photoconductive insulating layer on a conductive layer is first uniformly electrostatically charged. The imaging member is then exposed to a pattern of activating electromagnetic radiation, such as light. The radiation selectively dissipates the

charge on the illuminated areas of the photoconductive insulating layer while leaving behind an electrostatic latent image. This electrostatic latent image may then be developed to form a visible image by depositing charged particles of the same or opposite polarity on the surface of the photoconductive insulating layer. The resulting visible image may then be transferred from the imaging member directly or indirectly (such as by a transfer or other member) to a print substrate, such as transparency or paper. The imaging process may be repeated many times with reusable imaging members.

Common print quality issues are strongly dependent on the quality and interaction of these photoreceptor layers. For example, when a photoreceptor is used in combination with a contact charger and a toner obtained by chemical polymerization (polymerization toner), image quality may be deteriorated due to a surface of the photoreceptor being stained with a discharge product produced in contact charging or the polymerization toner remaining after a cleaning step. Still further, repetitive cycling causes the outermost layer of the photoreceptor to experience a high degree of frictional contact with other machine subsystem components used to clean and/or prepare the photoreceptor for imaging during each cycle. When repeatedly subjected to cyclic mechanical interactions against the machine subsystem components, a photoreceptor can experience severe frictional wear at the outermost organic photoreceptor layer surface that can greatly reduce the useful life of the photoreceptor. Ultimately, the resulting wear impairs photoreceptor performance and thus image quality. Another type of common image defect is thought to result from the accumulation of charge somewhere in the photoreceptor. Consequently, when a sequential image is printed, the accumulated charge results in image density changes in the current printed image that reveals the previously printed image. In the xerographic process spatially varying amounts of positive charges from the transfer station find themselves on the photoreceptor surface. If this variation is large enough it will manifest itself as a variation in the image potential in the following xerographic cycle and print out as a defect.

A conventional approach to photoreceptor life extension is to apply an overcoat layer with wear resistance. For bias charge roller (BCR) charging systems, overcoat layers are associated with a trade-off between A-zone deletion (i.e. an image defect occurring in A-zone: 28° C., 85% RH) and photoreceptor wear rate. For example, most organic photoconductor (OPC) materials sets require a certain level of wear rate in order to suppress A-zone deletion, thus limiting the life of a photoreceptor. The present embodiments, however, have demonstrated a decrease in wear rate of a photoreceptor while maintaining the image quality of the photoreceptor, such as decreased image deletions. The present embodiments provide photoreceptor technology for BCR charging systems with a significantly expanded life.

Roller-type applicators to continuously apply functional material (such as paraffin oil) to the surface of the photoreceptor are disclosed in patent applications, U.S. Ser. No. 13/279,981 and U.S. Ser. No. 13/326,414 incorporated in their entirety by reference herein. The applied thin layer of functional material addresses A-zone deletion, alleviates chattering of the cleaning blade, and reduces toner/additive contamination on the BCR. However, roller type applicators present issues. It is difficult to control the contact force of the roller against the surface of the photoreceptor or the BCR along the entire length during rotation, which affects the rate of diffusion of oil from the delivery roller and results in an uneven distribution of oil, particularly at the two ends of the photoreceptor or BCR surface. As a result, after several prints, toner density across a page becomes uneven, thus the edges of

the images sometimes become darker than the middle due to an excess amount of delivered oil. This can further cause the delivery roller to become contaminated with toner and additives over time due to inefficient cleaning of the surface of the photoreceptor (P/R) by the cleaning blade. Toner particles are eventually transferred to and contaminate the surface of the BCR.

Disclosed herein is a blade type applicator that can apply an ultra-thin layer of a functional material, such as paraffin oil, onto the surface of a P/R surface. The blade is positioned in a trailing configuration. The blade type applicator minimizes the problems associated with the roller-type applicator, in that the contact force of a blade can be more evenly distributed with less variance over the length of the P/R surface. The contact force is easily addressed intrinsically by adjusting the mechanical properties of the material, and/or the angle at which the blade contacts the P/R surface. A blade configuration offers other advantages over a roller configuration, such as: i) a more compact size, ii) reduced cost and fabrication complexity, and iii) a simpler geometry which makes it easier for optimization and integration into other systems.

A blade applicator 35 is shown in FIG. 3, and possesses the following characteristics. The blade applicator 35 is in a trailing position with respect the surface of the photoreceptor 34. The blade applicator 35 can be held in the trailing position by a holding mechanism such as a bracket 31 and blade clamp 33. The trailing position means the surface of the P/R pulls the blade applicator 35 as the P/R rotates. The blade clamp 33 has saw tooth grooves to fix the blade applicator 35 in place. The metal blade bracket 31 can be made of metal or plastic, and magnetically or mechanically attached to the housing of the P/R.

The blade applicator 35 is comprised of an elastomeric matrix having functional materials such as paraffin oil dispersed therein. The functional material diffuses through the elastomeric matrix onto an P/R surface. The metering of functional material can be controlled by the contact pressure between the blade and the surface of the P/R.

In the configuration shown in FIG. 3, the blade applicator 35 reduces A-zone deletion and high friction during longer-term printing, extending the life of the photoreceptor. Effective suppression of contamination on the BCR associated with low wear overcoated P/Rs is also provided by the blade applicator 35. The blade applicator 35 is compact in size, inexpensive and easily implemented.

In FIG. 4, there is illustrated an image-forming apparatus in a BCR charging system. As shown, the image-forming apparatus comprises a photoreceptor 34, a BCR 46 and a blade applicator 35. The blade applicator 35 contacts the photoreceptor 34 to deliver an ultra-thin layer of a functional material onto the surface of the photoreceptor 34. Subsequently, the photoreceptor 34 is substantially uniformly charged by the BCR 46 to initiate the electrophotographic reproduction process. The charged photoreceptor 34 is then exposed to a light image to create an electrostatic latent image on the photoreceptive member (not shown). This latent image is subsequently developed into a visible image by a toner developer 40. Thereafter, the developed toner image is transferred from the photoreceptor 34 through a record medium to a copy sheet or some other image support substrate to which the image may be permanently affixed for producing a reproduction of the original document (not shown). The photoreceptor surface is generally then cleaned with a cleaner 42 to remove any residual developing material therefrom, in preparation for successive imaging cycles.

In FIG. 5, there is illustrated an alternate embodiment image-forming apparatus in a BCR charging system. As

shown, the image-forming apparatus comprises a photoreceptor 34, a BCR 46 and a blade applicator 35. The blade applicator 35 contacts the BCR 46 which in turn contacts the photoreceptor 34 to deliver an ultra-thin layer of a functional material onto the surface of the photoreceptor 34. The photoreceptor 34 is substantially uniformly charged by the BCR 46 to initiate the electrophotographic reproduction process. The charged photoreceptor is then exposed to a light image to create an electrostatic latent image on the photoreceptive member (not shown). This latent image is subsequently developed into a visible image by a toner developer 40. Thereafter, the developed toner image is transferred from the photoreceptor member through a record medium to a copy sheet or some other image support substrate to which the image may be permanently affixed for producing a reproduction of the original document (not shown). The photoreceptor surface is generally then cleaned with a cleaner 42 to remove any residual developing material therefrom in preparation for successive imaging cycles.

In an embodiment of the blade applicator 35 shown in FIG. 6, the components of the system comprising the blade applicator 35 include single layer 63 of an elastomeric matrix 61 having pores or a porous material 62. The functional material is dispersed in the pores or the porous material 62 of layer 63. In embodiments, the blade applicator 35 includes a porous material rather than pores 42 to hold the functional material.

In an embodiment of the blade applicator shown in FIG. 7 there is a second layer 64 formed of an elastomeric material to meter the functional material to the surface of the P/R or BCR. The layer 64 is in a trailing position to the surface of the P/R 34. The layer 64 is disposed on layer 63. In FIG. 7 the blade applicator 35 includes a layer 63 and an elastomeric matrix 61 having pores or a porous material 62. The functional material is dispersed in the pores or the porous material 62 of layer 63. In embodiments, the blade applicator 35 can include a porous material rather than pores to hold the functional material.

In an embodiment of the blade applicator shown in FIG. 8 there is a second layer 64 formed of an elastomeric material to meter the functional material to the surface of the P/R or BCR. The second layer 64 surrounds the layer 63. The second layer 64 controls the delivery of functional material to surface of the photoreceptor or the BCR. In FIG. 8 the blade applicator 35 includes a layer 63 and an elastomeric matrix 61 having pores or a porous material 62. The functional material is dispersed in the pores or the porous material 62 of layer 63. The concentration of functional material is greater in layer 63 than in second layer 64.

The contact force of the edge of the blade applicator in contact with the P/R surface across the whole contact length can be controlled. In embodiments, a contact force of from about 10 g to about 60 g, or from about 15 g to about 50 g or from about 15 g to about 40 g is achieved. The contact force between the blade and the P/R can be easily adjusted by changing the stiffness of the material, the angle of contact, and/or the geometry of the blade.

In the embodiment shown in FIGS. 6, 7 and 8, the thickness of the blade applicator 35 may be varied depending on the application requirements. In specific embodiments, the thickness of the blade applicator is from about 0.1 mm to about 50 mm. In embodiments, the thickness of blade applicator is from about 1 mm to about 30 mm, or from about 5 mm to about 25 mm. In embodiments shown in FIGS. 7 and 8, the thickness of layer 64 is from about 0.01  $\mu\text{m}$  to about 5 mm.

The geometry of the tip of blade 35 may be shaped. Shown in FIG. 9 are various embodiments viewed in cross section for the shape of the tip 90 of blade 35. These include a polygonal

prism, a triangular prism, a cuboid, or a sphere. The orientation of the tip shape can be varied.

In embodiments the layer 63 has pores of a size from about 10 nm to about 100  $\mu\text{m}$ , or from about 20 nm to about 50  $\mu\text{m}$  or from about 50 nm to about 10  $\mu\text{m}$ . In the embodiment shown in FIGS. 7 and 8, layer 64 has pores of less than about 1  $\mu\text{m}$ , or less than about 500 nm or less than about 300 nm or less than 100 nm or less than 50 nm. The blade applicator 35 may have a geometry at the leading edge of the blade contacting the P/R surface. The geometry shown is that of a right angle, however, in embodiments the leading edge may be shaped.

In embodiments the layer 63 has a porous material 62 dispersed in the elastomer 61. The porous material 62 has a porosity of from about 50 percent to about 99.9 percent. The porous material functions as a reservoir to store the functional material. The pores of the porous material are from about 2 nm up to about 50 microns, or the pores are from about 10 nm microns to about 20 microns, or the pores are from about 100 nm to about 17 microns. The pores of the porous material are filled with functional material. When layer 64 is provided in a blade applicator, the layer 64 can help control the diffusion of the functional material from the layer comprising the elastomeric material and functional material. The blade applicator applies an ultra-thin film of functional material to the surface of a photoreceptor either directly or indirectly which: i) reduces friction between the P/R and the cleaning blade and ii) eliminates A-zone deletions, both of which improve image quality.

The incorporation of a solid, porous material, for example silica aerogel, increases the amount of functional material (particularly one that is incompatible with the elastomeric matrix) stored in the delivery roller. Paraffin oil and PDMS are immiscible, which limits the quantity of paraffin oil that can be dispersed in a PDMS matrix to about 33 weight percent of the layer. Silica aerogels, which can have porosities up to 99.9 percent, absorb paraffin oil and stabilize its dispersion in the elastomeric matrix. The delivery roller described herein provides a way to store larger quantities of functional material in the delivery roller and increase its overall lifetime.

The present embodiments employ a delivery apparatus and system to deliver a layer of functional materials onto the photoreceptor surface either directly or through a charging roller. The functional material is applied to the photoreceptor surface and acts as lubricant and/or a barrier against moisture and surface contaminants and improves xerographic performance in high humidity conditions, such as, for example, A-zone environment. The ultra-thin layer may be provided on a nano-scale or molecular level.

In embodiments, there is provided an image forming apparatus that includes a blade applicator for delivering functional materials onto a photoreceptor. The apparatus typically comprises an imaging member; a charging unit comprising a charging roller disposed in contact with the surface of the imaging member; and a delivery unit disposed in contact with the surface of the charging roller, wherein the blade applicator applies a layer of functional material to the surface of the charging roller and the charging roller in turn applies a layer of the functional material onto the surface of the imaging member. In an embodiment, the blade applicator delivers a functional material directly to the surface of the imaging member.

In the present embodiments, the functional material contains with pores or porous material 62 of layer 63 of the blade applicator 35 and is delivered to the surface of the photoreceptor (FIG. 4) or the functional material is delivered to the surface of BCR 46 (FIG. 5). The functional material is trans-

ferred to the surface of the imaging member directly (FIG. 4) or indirectly through transfer to the BCR surface (FIG. 5). Blade applicators fabricated according to the present embodiments have been shown to contain sufficient quantities of the functional material to continuously supply an ultra-thin layer of the functional material to the surface of the BCR/photoreceptor.

In embodiments, the functional material can be an organic or inorganic compound, oligomer or polymer, or a mixture thereof. The functional materials may be in the form of liquid, wax, or gel, and a mixture thereof. The functional material may also be selected from the group consisting of a lubricant material, a hydrophobic material, an oleophobic material, an amphiphilic material, and mixtures thereof. Illustrative examples of functional materials may include, for example, a liquid material selected from the group consisting of hydrocarbons, fluorocarbons, mineral oil, synthetic oil, natural oil, and mixtures thereof. The functional materials may further contain a functional group that facilitates adsorption of the functional materials on the photoreceptor surface, and optionally a reactive group that can chemically modify the photoreceptor surface. For examples, the functional materials may comprise paraffinic compound, alkanes, fluoroalkanes, alkyl silanes, fluoroalkyl silanes alkoxy-silanes, siloxanes, glycols or polyglycols, mineral oil, synthetic oil, natural oil or mixture thereof.

In embodiments, the blade applicator 35 in FIG. 6 or FIG. 7 may be comprised of a polymer selected from the group consisting of polysiloxanes, polyurethanes, polyesters, fluoro-silicones, polyolefin, fluoroelastomers, synthetic rubber, natural rubber, and mixtures thereof.

The porous material 42 is selected from the group consisting of aerogel particles, ceramic particles, polymers, foam wood and glass. The porosity of the porous material 42 is from about 50 percent to about 99.9 percent. In embodiments the porosity of the porous material is from about 60 percent to about 99 percent, or from about 65 percent to about 95 percent. The porous material and functional material comprise about 50 weight percent to about 90 weight percent of the blade applicator 35. In embodiments, the porous material and functional material comprise about 55 weight percent to about 85 weight percent of layer 63, or the porous material and functional material comprise about 60 weight percent to about 80 weight percent of layer 63.

Aerogels may be described, in general terms, as gels that have been dried to a solid phase by removing pore fluid and replacing the pore fluid with air. As used herein, an "aerogel" refers to a material that is generally a very low density ceramic solid, typically formed from a gel. The term "aerogel" is thus used to indicate gels that have been dried so that the gel shrinks little during drying, preserving its porosity and related characteristics. In contrast, "hydrogel" is used to describe wet gels in which pore fluids are aqueous fluids. The term "pore fluid" describes fluid contained within pore structures during formation of the pore element(s). Upon drying, such as by supercritical drying, aerogel particles are formed that contain a significant amount of air, resulting in a low density solid and a high surface area. In various embodiments, aerogels are thus low-density microcellular materials characterized by low mass densities, large specific surface areas and very high porosities. In particular, aerogels are characterized by their unique structures that comprise a large number of small inter-connected pores. After the solvent is removed, the polymerized material is pyrolyzed in an inert atmosphere to form the aerogel.

Any suitable aerogel component can be used. In embodiments, the aerogel component can be, for example, selected

from inorganic aerogels, organic aerogels, carbon aerogels, and mixtures thereof. In particular embodiments, ceramic aerogels can be suitably used. These aerogels are typically composed of silica, but may also be composed of metal oxides, such as alumina, titania and zirconia, or carbon, and can optionally be doped with other elements such as a metal. In some embodiments, the aerogel component can comprise aerogels chosen from polymeric aerogels, colloidal aerogels, and mixtures thereof.

10 Aerogel particles of embodiments may have porosities of from about 50 percent to about 99.9 percent, in which the aerogel can contain 99.9 percent empty space. In embodiments the aerogel particles have porosities of from about 50 percent to about 99.0 percent, or from 50 percent to about 98 percent. In embodiments, the pores of aerogel components may have diameters of from about 2 nm to about 500 nm, or from about 10 nm to about 400 nm or from about 20 nm to about 100 nm. In particular embodiments, aerogel components may have porosities of more than 50% pores with 15 diameters of less than 100 nm and even less than about 20 nm. In embodiments, the aerogel components may be in the form of particles having a shape that is spherical, or near-spherical, cylindrical, rod-like, bead-like, cubic, platelet-like, and the like.

20 In embodiments, the aerogel components include aerogel particles, powders, or dispersions ranging in average volume particle size of from about 1  $\mu\text{m}$  to about 100  $\mu\text{m}$ , or about 3  $\mu\text{m}$  to about 50  $\mu\text{m}$ , or about 5  $\mu\text{m}$  to 20  $\mu\text{m}$ . The aerogel components can include aerogel particles that appear as well 25 dispersed single particles or as agglomerates of more than one particle or groups of particles within the polymer material.

Generally, the type, porosity, pore size, and amount of aerogel used for a particular embodiment may be chosen based upon the desired properties of the resultant composition 30 and upon the properties of the polymers and solutions thereof into which the aerogel is being combined. For example, if a pre-polymer (such as a low molecular weight polyurethane monomer that has a relatively low process viscosity, for example less than 10 centistokes) is chosen for use 35 in an embodiment, then a high porosity, for example greater than 80%, and high specific surface area, for example greater than about 500  $\text{m}^2/\text{gm}$ , aerogel having relatively small pore size, for example less than about 100 nm, may be mixed at relatively high concentrations, for example greater than about 40 2 weight percent to about 20 weight percent, into the pre-polymer by use of moderate-to-high energy mixing techniques, for example by controlled temperature, high shear and/or blending. If a hydrophilic-type aerogel is used, upon cross-linking and curing/post curing the pre-polymer to form 45 an infinitely long matrix of polymer and aerogel filler, the resultant composite may exhibit improved hydrophobicity and increased hardness when compared to a similarly prepared sample of unfilled polymer. The improved hydrophobicity may be derived from the polymer and aerogel interacting 50 during the liquid-phase processing whereby a portion of the molecular chain of the polymer interpenetrates into the pores of the aerogel and the non-pore regions of the aerogel 55 serves to occupy some or all of the intermolecular space where water molecules could otherwise enter and occupy.

60 Aerogels that can suitably be used in embodiments may be divided into three major categories: inorganic aerogels, organic aerogels and carbon aerogels.

Inorganic aerogels, such as silica aerogels, are generally 65 formed by sol-gel polycondensation of metal oxides to form highly cross-linked, transparent hydrogels. These hydrogels are subjected to supercritical drying to form inorganic aerogels.

## 11

Organic aerogels are generally formed by sol-gel polycondensation of resorcinol and formaldehyde. These hydrogels are subjected to supercritical drying to form organic aerogels.

Carbon aerogels are generally formed by pyrolyzing organic aerogels in an inert atmosphere. Carbon aerogels are composed of covalently bonded, nanometer-sized particles that are arranged in a three-dimensional network. Carbon aerogels, unlike high surface area carbon powders, have oxygen-free surfaces, which can be chemically modified to increase their compatibility with polymer matrices.

For example, in one embodiment, the aerogel particles can be a silica silicate having an average particle size of 5-15 microns, a porosity of 90% or more, a bulk density of 40-100 kg/m<sup>3</sup>, and a surface area of 600-800 m<sup>2</sup>/g. Of course, materials having one or properties outside of these ranges can be used, as desired.

In general, a wide range of aerogel components are known in the art and have been applied in a variety of uses. One specific non-limiting example is the commercially available powder that has already been chemically treated, Dow Corning VM-2270 Aerogel fine particles having a size of about 5-15 microns.

In embodiments, the blade applicator 35 contains an elastomeric matrix comprised of a polymer selected from the group consisting of polysiloxane, silicones, polyurethane, polyester, fluoro-silicone, polyolefin, fluoroelastomer, synthetic rubber, natural rubber and mixtures thereof.

In embodiments, the blade applicator 35 in FIG. 6 is an elastomeric material cast with the porous material 62 by use of a mold. Thereafter, the elastomeric matrix is cured. The blade applicator 35 is impregnated with a functional material, such as paraffin by immersion. After curing, the elastomeric matrix containing the porous material and functional material is extracted from the mold. In embodiments (FIG. 7), a layer 64 is prepared by mixing a cross-linkable elastomeric polymer and then casting the mixture onto a surface of the blade applicator 35 by use of a mold. The elastomeric material is then cured to form the delivery member.

In a specific embodiment, the blade applicator 35 is a paraffin-impregnated PDMS that includes the porous material 62. The blade applicator 35 of paraffin-impregnated silicone is prepared by mixing paraffin into a cross-linkable polydimethylsiloxane (PDMS) and the porous material 62, such as aerogel particles, and then casting the mixture by use of a mold. Thereafter, the PDMS is cured. The blade applicator 35 is impregnated with a functional material, such as paraffin by immersion. After curing, the blade applicator 35 is removed from the mold. In embodiments, the layer 64 is prepared by mixing a cross-linkable polydimethylsiloxane (PDMS) and then casting the mixture into the blade applicator 35 by use of a mold. In embodiments, the liquid cross-linkable PDMS is prepared from a two-component system, namely, a base agent and a curing agent. In further embodiments, the base agent and curing agent are present in a weight ratio of from about 50:1 to about 2:1, or from about 20:1 to about 5:1 in both layers 63 and 64. In embodiments, the weight ratio of the elastomeric material to the porous material and functional material of the layer 63 is at a weight ratio of from about 20:1 to about 1:5, or from about 10:1 to about 1:5 or from about 3:1 to about 1:3.

The description below describes embodiments of photoconductors

#### The Overcoat Layer

Other layers of the imaging member may include, for example, an optional over coat layer 32. The optional overcoat layer 32, if desired, may be disposed over the charge transport layer 20 to provide imaging member surface pro-

## 12

tection as well as improve resistance to abrasion. In embodiments, the overcoat layer 32 may have a thickness ranging from about 0.1 micrometer to about 15 micrometers or from about 1 micrometer to about 10 micrometers, or in a specific embodiment, about 3 micrometers to about 10 micrometers. These overcoating layers typically comprise a charge transport component and an optional organic polymer or inorganic polymer. These overcoating layers may include thermoplastic organic polymers or cross-linked polymers such as thermosetting resins, UV or e-beam cured resins, and the like. The overcoat layers may further include a particulate additive such as metal oxides including aluminum oxide and silica, or low surface energy polytetrafluoroethylene (PTFE), and combinations thereof.

Any known or new overcoat materials may be included for the present embodiments. In embodiments, the overcoat layer may include a charge transport component or a cross-linked charge transport component. In particular embodiments, for example, the overcoat layer comprises a charge transport component comprised of a tertiary arylamine containing a substituent capable of self cross-linking or reacting with the polymer resin to form a cured composition. Specific examples of charge transport components suitable for overcoat layer comprise the tertiary arylamine with a general formula of



wherein Ar<sup>1</sup>, Ar<sup>2</sup>, Ar<sup>3</sup>, and Ar<sup>4</sup> each independently represents an aryl group having about 6 carbon atoms to about 30 carbon atoms, Ar<sup>5</sup> represents aromatic hydrocarbon group having about 6 carbon atoms to about 30 carbon atoms, and k represents 0 or 1, and wherein at least one of Ar<sup>1</sup>, Ar<sup>2</sup>, Ar<sup>3</sup>, Ar<sup>4</sup>, and Ar<sup>5</sup> comprises a substituent selected from the group consisting of hydroxyl (—OH), a hydroxymethyl (—CH<sub>2</sub>OH), an alkoxyethyl (—CH<sub>2</sub>OR, wherein R is an alkyl having 1 carbon atoms to about 10 carbons), a hydroxylalkyl having 1 carbon atoms to about 10 carbons, and mixtures thereof. In other embodiments, Ar<sup>1</sup>, Ar<sup>2</sup>, Ar<sup>3</sup>, and Ar<sup>4</sup> each independently represent a phenyl or a substituted phenyl group, and Ar<sup>5</sup> represents a biphenyl or a terphenyl group.

#### The Substrate

The photoreceptor support substrate 10 may be opaque or substantially transparent, and may comprise any suitable organic or inorganic material having the requisite mechanical properties. The entire substrate can comprise the same material as that in the electrically conductive surface, or the electrically conductive surface can be merely a coating on the substrate. Any suitable electrically conductive material can be employed, such as for example, metal or metal alloy. Electrically conductive materials include copper, brass, nickel, zinc, chromium, stainless steel, conductive plastics and rubbers, aluminum, semitransparent aluminum, steel, cadmium, silver, gold, zirconium, niobium, tantalum, vanadium, hafnium, titanium, nickel, niobium, stainless steel, chromium, tungsten, molybdenum, paper rendered conductive by the inclusion of a suitable material therein or through conditioning in a humid atmosphere to ensure the presence of sufficient water content to render the material conductive, indium, tin, metal oxides, including tin oxide and indium tin

oxide, and the like. It could be a single metallic compound or dual layers of different metals and/or oxides.

The substrate **10** can also be formulated entirely of an electrically conductive material, or it can be an insulating material including inorganic or organic polymeric materials, such as MYLAR, a commercially available biaxially oriented polyethylene terephthalate from DuPont, or polyethylene naphthalate available as KALEDEX 2000, with a ground plane layer **12** comprising a conductive titanium or titanium/zirconium coating, otherwise a layer of an organic or inorganic material having a semiconductive surface layer, such as indium tin oxide, aluminum, titanium, and the like, or exclusively be made up of a conductive material such as, aluminum, chromium, nickel, brass, other metals and the like. The thickness of the support substrate depends on numerous factors, including mechanical performance and economic considerations.

The substrate **10** may have a number of many different configurations, such as for example, a plate, a cylinder, a drum, a scroll, an endless flexible belt, and the like. In the case of the substrate being in the form of a belt, as shown in FIG. 2, the belt can be seamed or seamless. In embodiments, the photoreceptor herein is in a drum configuration.

The thickness of the substrate **10** depends on numerous factors, including flexibility, mechanical performance, and economic considerations. The thickness of the support substrate **10** of the present embodiments may be at least about 500 micrometers, or no more than about 3,000 micrometers, or be at least about 750 micrometers, or no more than about 2500 micrometers.

#### The Ground Plane

The electrically conductive ground plane **12** may be an electrically conductive metal layer which may be formed, for example, on the substrate **10** by any suitable coating technique, such as a vacuum depositing technique. Metals include aluminum, zirconium, niobium, tantalum, vanadium, hafnium, titanium, nickel, stainless steel, chromium, tungsten, molybdenum, and other conductive substances, and mixtures thereof. The conductive layer may vary in thickness over substantially wide ranges depending on the optical transparency and flexibility desired for the electrophotocuctive member. Accordingly, for a flexible photoresponsive imaging device, the thickness of the conductive layer may be at least about 20 Angstroms, or no more than about 750 Angstroms, or at least about 50 Angstroms, or no more than about 200 Angstroms for an optimum combination of electrical conductivity, flexibility and light transmission.

#### The Hole Blocking Layer

After deposition of the electrically conductive ground plane layer, the hole blocking layer **14** may be applied thereto. Electron blocking layers for positively charged photoreceptors allow holes from the imaging surface of the photoreceptor to migrate toward the conductive layer. For negatively charged photoreceptors, any suitable hole blocking layer capable of forming a barrier to prevent hole injection from the conductive layer to the opposite photoconductive layer may be utilized. The hole blocking layer may include polymers such as polyvinylbutyral, epoxy resins, polyesters, polysiloxanes, polyamides, polyurethanes and the like, or may be nitrogen containing siloxanes or nitrogen containing titanium compounds such as trimethoxysilyl propylene diamine, hydrolyzed trimethoxysilyl propyl ethylene diamine, N-beta-(aminoethyl)gamma-amino-propyl trimethoxy silane, isopropyl 4-aminobenzene sulfonyl, di(dodecylbenzene sulfonyl)titanate, isopropyl di(4-aminobenzoyl)isostearoyl titanate, isopropyl tri(N-ethylamino-ethylamino)titanate, isopropyl trianthranil titanate, isopropyl tri(N,N-dimethyl-

ethylamino)titanate, titanium-4-amino benzene sulfonate oxyacetate, titanium 4-aminobenzoate isostearate oxyacetate,  $[H_2N(CH_2)_4]CH_3Si(OCH_3)_2$ , (gamma-aminobutyl) methyl diethoxysilane, and  $[H_2N(CH_2)_3]CH_3Si(OCH_3)_2$  5 (gamma-aminopropyl)methyl diethoxysilane.

General embodiments of the undercoat layer may comprise a metal oxide and a resin binder. The metal oxides that can be used with the embodiments herein include, but are not limited to, titanium oxide, zinc oxide, tin oxide, aluminum oxide, 10 silicon oxide, zirconium oxide, indium oxide, molybdenum oxide, and mixtures thereof. Undercoat layer binder materials may include, for example, polyesters, MOR-ESTER 49,000 from Morton International Inc., VITEL PE-100, VITEL PE-200, VITEL PE-200D, and VITEL PE-222 from Good-year Tire and Rubber Co., polyarylates such as ARDEL from AMOCO Production Products, polysulfone from AMOCO Production Products, polyurethanes, and the like.

The hole blocking layer should be continuous and have a thickness of less than about 0.5 micrometer because greater 20 thicknesses may lead to undesirably high residual voltage. A hole blocking layer of between about 0.005 micrometer and about 0.3 micrometer is used because charge neutralization after the exposure step is facilitated and optimum electrical 25 performance is achieved. A thickness of between about 0.03 micrometer and about 0.06 micrometer is used for hole blocking layers for optimum electrical behavior. The hole blocking layers that contain metal oxides such as zinc oxide, titanium oxide, or tin oxide, may be thicker, for example, having a thickness up to about 25 micrometers. The blocking layer 30 may be applied by any suitable conventional technique such as spraying, dip coating, draw bar coating, gravure coating, silk screening, air knife coating, reverse roll coating, vacuum deposition, chemical treatment and the like. For convenience in obtaining thin layers, the blocking layer is applied in the 35 form of a dilute solution, with the solvent being removed after deposition of the coating by conventional techniques such as by vacuum, heating and the like. Generally, a weight ratio of between about 0.05:100 to about 0.5:100 for the hole blocking layer material and solvent is satisfactory for spray coating.

#### The Charge Generation Layer

The charge generation layer **18** may thereafter be applied to the undercoat layer **14**. Any suitable charge generation binder including a charge generating/photoconductive material, 45 which may be in the form of particles and dispersed in a film forming binder, such as an inactive resin, may be utilized. Examples of charge generating materials include, for example, inorganic photoconductive materials such as amorphous selenium, trigonal selenium, and selenium alloys selected from the group consisting of selenium-tellurium, 50 selenium-tellurium-arsenic, selenium arsenide and mixtures thereof, and organic photoconductive materials including various phthalocyanine pigments such as the X-form of metal free phthalocyanine, metal phthalocyanines such as vanadyl phthalocyanine and copper phthalocyanine, hydroxy gallium phthalocyanines, chlorogallium phthalocyanines, titanyl phthalocyanines, quinacridones, dibromo anthanthrone pigments, benzimidazole perylene, substituted 2,4-diamino-triazines, polynuclear aromatic quinones, enzimidazole 55 perylene, and the like, and mixtures thereof, dispersed in a film forming polymeric binder. Selenium, selenium alloy, benzimidazole perylene, and the like and mixtures thereof may be formed as a continuous, homogeneous charge generation layer. Benzimidazole perylene compositions are well known and described, for example, in U.S. Pat. No. 4,587, 60 189, the entire disclosure thereof being incorporated herein by reference. Multi-charge generation layer compositions

## 15

may be used where a photoconductive layer enhances or reduces the properties of the charge generation layer. Other suitable charge generating materials known in the art may also be utilized, if desired. The charge generating materials selected should be sensitive to activating radiation having a wavelength between about 400 nm and about 900 nm during the imagewise radiation exposure step in an electrophotographic imaging process to form an electrostatic latent image. For example, hydroxygallium phthalocyanine absorbs light of a wavelength of from about 370 nm to about 950 nm, as disclosed, for example, in U.S. Pat. No. 5,756,245, the entire disclosure thereof being incorporated herein by reference.

Any suitable inactive resin materials may be employed as a binder in the charge generation layer **18**, including those described, for example, in U.S. Pat. No. 3,121,006, the entire disclosure thereof being incorporated herein by reference. Organic resinous binders include thermoplastic and thermosetting resins such as one or more of polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl butyral, polyvinyl acetate, polysiloxanes, polyacrylates, polyvinyl acetals, polyamides, polyimides, amino resins, phenylene oxide resins, terephthalic acid resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride/vinylchloride copolymers, vinylacetate/vinylidene chloride copolymers, styrene-alkyd resins, and the like. Another film-forming polymer binder is PCZ-400 (poly(4,4'-dihydroxy-diphenyl-1-1-cyclohexane) which has a viscosity-molecular weight of 40,000 and is available from Mitsubishi Gas Chemical Corporation (Tokyo, Japan).

The charge generating material can be present in the resinous binder composition in various amounts. Generally, at least about 5 percent by volume, or no more than about 90 percent by volume of the charge generating material is dispersed in at least about 95 percent by volume, or no more than about 10 percent by volume of the resinous binder, and more specifically at least about 20 percent, or no more than about 60 percent by volume of the charge generating material is dispersed in at least about 80 percent by volume, or no more than about 40 percent by volume of the resinous binder composition.

In specific embodiments, the charge generation layer **18** may have a thickness of at least about 0.1  $\mu\text{m}$ , or no more than about 2  $\mu\text{m}$ , or of at least about 0.2  $\mu\text{m}$ , or no more than about 1  $\mu\text{m}$ . These embodiments may be comprised of chlorogallium phthalocyanine or hydroxygallium phthalocyanine or mixtures thereof. The charge generation layer **18** containing the charge generating material and the resinous binder material generally ranges in thickness of at least about 0.1  $\mu\text{m}$ , or no more than about 5  $\mu\text{m}$ , for example, from about 0.2  $\mu\text{m}$  to about 3  $\mu\text{m}$  when dry. The charge generation layer thickness is generally related to binder content. Higher binder content compositions generally employ thicker layers for charge generation.

#### The Charge Transport Layer

In a drum photoreceptor, the charge transport layer comprises a single layer of the same composition. As such, the charge transport layer will be discussed specifically in terms of a single layer **20**, but the details will be also applicable to an embodiment having dual charge transport layers. The charge transport layer **20** is thereafter applied over the charge generation layer **18** and may include any suitable transparent

## 16

organic polymer or non-polymeric material capable of supporting the injection of photogenerated holes or electrons from the charge generation layer **18** and capable of allowing the transport of these holes/electrons through the charge transport layer to selectively discharge the surface charge on the imaging member surface. In one embodiment, the charge transport layer **20** not only serves to transport holes, but also protects the charge generation layer **18** from abrasion or chemical attack and may therefore extend the service life of the imaging member. The charge transport layer **20** can be a substantially non-photoconductive material, but one which supports the injection of photogenerated holes from the charge generation layer **18**.

The charge transport layer **20** is normally transparent in a wavelength region in which the electrophotographic imaging member is to be used when exposure is affected there to ensure that most of the incident radiation is utilized by the underlying charge generation layer **18**. The charge transport layer **20** should exhibit excellent optical transparency with negligible light absorption and no charge generation when exposed to a wavelength of light useful in xerography, e.g., 400 nm to 900 nm. In the case when the photoreceptor is prepared with the use of a transparent substrate **10** and also a transparent or partially transparent conductive layer **12**, imagewise exposure or erasure may be accomplished through the substrate **10** with all light passing through the back side of the substrate **10**. In this case, the materials of the charge transport layer **20** need not transmit light in the wavelength region of use if the charge generation layer **18** is sandwiched between the substrate **10** and the charge transport layer **20**. The charge transport layer **20** in conjunction with the charge generation layer **18** is an insulator to the extent that an electrostatic charge placed on the charge transport layer **20** is not conducted in the absence of illumination. The charge transport layer **20** should trap minimal charges as the charge passes through it during the discharging process.

The charge transport layer **20** may include any suitable charge transport component or activating compound useful as an additive dissolved or molecularly dispersed in an electrically inactive polymeric material, such as a polycarbonate binder, to form a solid solution and thereby making this material electrically active. "Dissolved" refers, for example, to forming a solution in which the small molecule is dissolved in the polymer to form a homogeneous phase; and molecularly dispersed in embodiments refers, for example, to charge transporting molecules dispersed in the polymer, the small molecules being dispersed in the polymer on a molecular scale. The charge transport component may be added to a film forming polymeric material which is otherwise incapable of supporting the injection of photogenerated holes from the charge generation material and incapable of allowing the transport of these holes. This addition converts the electrically inactive polymeric material to a material capable of supporting the injection of photogenerated holes from the charge generation layer **18** and capable of allowing the transport of these holes through the charge transport layer **20** in order to discharge the surface charge on the charge transport layer **20**. The high mobility charge transport component may comprise small molecules of an organic compound which cooperate to transport charge between molecules and ultimately to the surface of the charge transport layer **20**. For example, but not limited to, N,N'-diphenyl-N,N'-bis(3-methyl phenyl)-1,1'-biphenyl-4,4'-diamine (TPD), other arylamines like triphenyl amine, N,N,N',N'-tetra-p-tolyl-1,1'-biphenyl-4,4'-diamine (TM-TPD), and the like.

A number of charge transport compounds can be included in the charge transport layer, which layer generally is of a

thickness of from about 5 micrometers to about 75 micrometers, and more specifically, of a thickness of from about 15 micrometers to about 40 micrometers. Examples of charge transport components are aryl amines.

Examples of the binder materials selected for the charge transport layers include components, such as those described in U.S. Pat. No. 3,121,006, the disclosure of which is totally incorporated herein by reference in its entirety. Specific examples of polymer binder materials include polycarbonates, polyarylates, acrylate polymers, vinyl polymers, cellulose polymers, polyesters, polysiloxanes, polyamides, polyurethanes, poly(cyclo olefins), and epoxies, and random or alternating copolymers thereof. In embodiments, the charge transport layer **20**, such as a hole transport layer, may have a thickness of at least about 10  $\mu\text{m}$ , or no more than about 40  $\mu\text{m}$ .

The charge transport layer **20** should be an insulator to the extent that the electrostatic charge placed on the hole transport layer is not conducted in the absence of illumination at a rate sufficient to prevent formation and retention of an electrostatic latent image thereon. The charge transport layer **20** is substantially nonabsorbing to visible light or radiation in the region of intended use, but is electrically "active" in that it allows the injection of photogenerated holes from the photoconductive layer, that is the charge generation layer, and allows these holes to be transported through itself to selectively discharge a surface charge on the surface of the active layer.

In addition, in the present embodiments using a belt configuration, the charge transport layer **20** may consist of a single pass charge transport layer or a dual pass charge transport layer (or dual layer charge transport layer) with the same or different transport molecule ratios. In these embodiments, the dual layer charge transport layer **20** has a total thickness of from about 10  $\mu\text{m}$  to about 40  $\mu\text{m}$ . In other embodiments, each layer of the dual layer charge transport layer may have an individual thickness of from 2  $\mu\text{m}$  to about 20  $\mu\text{m}$ . Moreover, the charge transport layer **20** may be configured such that it is used as a top layer of the photoreceptor to inhibit crystallization at the interface of the charge transport layer and the overcoat layer. In another embodiment, the charge transport layer **20** may be configured such that it is used as a first pass charge transport layer to inhibit microcrystallization occurring at the interface between the first pass and second pass layers.

#### The Adhesive Layer

An optional separate adhesive interface layer may be provided in certain configurations, such as for example, in flexible web configurations. In the embodiment illustrated in FIG. 1, the interface layer would be situated between the blocking layer **14** and the charge generation layer **18**. The interface layer may include a copolyester resin. Exemplary polyester resins which may be utilized for the interface layer include polyarylatepolyvinylbutyrals, such as ARDEL POLYARYLATE (U-100) commercially available from Toyota Hsutsu Inc., VITEL PE-100, VITEL PE-200, VITEL PE-200D, and VITEL PE-222, all from Bostik, 49,000 polyester from Rohm Hass, polyvinyl butyral, and the like. The adhesive interface layer may be applied directly to the hole blocking layer **14**. Thus, the adhesive interface layer in embodiments is in direct contiguous contact with both the underlying hole blocking layer **14** and the overlying charge generator layer **18** to enhance adhesion bonding to provide linkage. In yet other embodiments, the adhesive interface layer is entirely omitted.

The adhesive interface layer may have a thickness of at least about 0.01 micrometers, or no more than about 900

micrometers after drying. In embodiments, the dried thickness is from about 0.03 micrometers to about 1 micrometer. The Ground Strip

The ground strip **19** may comprise a film forming polymer binder and electrically conductive particles. Any suitable electrically conductive particles may be used in the electrically conductive ground strip layer **19**. The ground strip **19** may comprise materials which include those enumerated in U.S. Pat. No. 4,664,995 incorporated in its entirety by reference herein. Electrically conductive particles include carbon black, graphite, copper, silver, gold, nickel, tantalum, chromium, zirconium, vanadium, niobium, indium tin oxide and the like. The electrically conductive particles may have any suitable shape. Shapes may include irregular, granular, spherical, elliptical, cubic, flake, filament, and the like. The electrically conductive particles should have a particle size less than the thickness of the electrically conductive ground strip layer to avoid an electrically conductive ground strip layer having an excessively irregular outer surface. An average particle size of less than about 10 micrometers generally avoids excessive protrusion of the electrically conductive particles at the outer surface of the dried ground strip layer and ensures relatively uniform dispersion of the particles throughout the matrix of the dried ground strip layer. The concentration of the conductive particles to be used in the ground strip depends on factors such as the conductivity of the specific conductive particles utilized.

The ground strip **19** layer may have a thickness of at least about 7 micrometers, or no more than about 42 micrometers, or of at least about 14 micrometers, or no more than about 27 micrometers.

#### The Anti-Curl Back Coating Layer

The anti-curl back coating **1** may comprise organic polymers or inorganic polymers that are electrically insulating or slightly semi-conductive. The anti-curl back coating **1** provides flatness and/or abrasion resistance.

Anti-curl back coating **1** may be formed at the back side of the substrate **10**, opposite to the imaging layers. The anti-curl back coating **1** may comprise a film forming resin binder and an adhesion promoter additive. The resin binder may be the same resins as the resin binders of the charge transport layer discussed above. Examples of film forming resins include polyacrylate, polystyrene, bisphenol polycarbonate, poly(4, 4'-isopropylidene diphenyl carbonate), 4,4'-cyclohexylidene diphenyl polycarbonate, and the like. Adhesion promoters used as additives include 49,000 (du Pont), Vitel PE-100, Vitel PE-200, Vitel PE-307 (Goodyear), and the like. Usually from about 1 to about 15 weight percent adhesion promoter is selected for film forming resin addition. The thickness of the anti-curl back coating is at least about 3 micrometers, or no more than about 35 micrometers, or about 14 micrometers.

Various exemplary embodiments encompassed herein include a method of imaging which includes generating an electrostatic latent image on an imaging member, developing a latent image, and transferring the developed electrostatic image to a suitable substrate.

While embodiments have been illustrated with respect to one or more implementations, alterations and/or modifications can be made to the illustrated examples without departing from the spirit and scope of the appended claims. In addition, while a particular feature herein may have been disclosed with respect to only one of several implementations, such feature may be combined with one or more other features of the other implementations as may be desired and advantageous for any given or particular function.

#### EXAMPLES

A blade applicator was fabricated and tested. Polydimethylsiloxane (PDMS) was prepared from a two component,

19

commercially available system. The components were mixed in a 10:1 ratio of base to curing agent. Paraffin oil was added to the pre-polymer in a 1 to 2 ratio of oil to pre-polymer. The three components were thoroughly mixed together, and degassed in a vacuum desiccator for 30 minutes. The resulting emulsion was carefully injected into a rectangular mould (anodized aluminum) using a disposable syringe which was then cured for three hours at about 60° C. After curing, the blade applicator was extracted from the mould and mounted onto the blade bracket. The blade has thickness of about 5 mm, width of about 15 mm, and length of about 130 mm.

The modified imaging apparatus with the blade applicator and a low wear overcoated photoreceptor was conditioned in A-zone before machine testing. The print test was performed with the Xerox DocuColor 250 machine in A-zone (28° C., 85% RH) to evaluate image quality, specifically A-zone deletion and BCR contamination. Overcoated P/R drums generally fail to turn in machines in A-zone due to high friction/torque which results in motor fault. After installing the blade applicator onto the CRU, the motor could turn the overcoated drums indicating that paraffin oil was supplied from the blade to lubricate the system. The blade applicator was approximately 130 mm in length (shorter than the full length of the P/R) so that paraffin oil was only applied onto a portion of the photoreceptor and the other portion (with no paraffin) was used as a control. This allowed the comparison of the image quality of prints obtained simultaneously from regions with and without applied paraffin oil. FIG. 8 presents the results of the print tests after 10 kcycles. In FIG. 8, the control section (no contact with applicator and therefore no applied paraffin oil) has severe streaking in the image due to toner/additive contamination on the BCR and blade chattering. The control section also resulted in severe A-zone deletion (only 10 lines out of 13 lines can be recognized in this portion of FIG. 8). In contrast, there was a dramatic improvement in image quality developed from the paraffin-applied P/R surface area (all 13 lines can be recognized in this portion of FIG. 8). The applied paraffin layer also significantly lubricates the cleaning blade and helps suppress the toner/additive contamination on the BCR due to inefficient cleaning associated with the overcoated BCR. Additive accumulation diminishes the charging efficiency of BCR (with lower surface charging voltage). The prints show that the area of the BCR not in contact with the applicator was severely contaminated with toner and additives. The section of the BCR corresponding to the position of the blade applicator was clean and therefore those regions of the images were brighter than the control section under the same charging condition.

The tests demonstrated that the blade-type applicator was effective in suppressing A-zone deletion and reducing friction-induced blade chatter.

It will be appreciated that variants of the above-disclosed and other features and functions or alternatives thereof, may be combined into other different systems or applications. Various presently unforeseen or unanticipated alternatives, modifications, variations, or improvements therein may be subsequently made by those skilled in the art which are also encompassed by the following claims.

What is claimed is:

1. An applicator for use in an image forming apparatus comprising:  
a blade applicator comprising an elastomeric matrix, a functional material and aerogel particles, the functional material and the aerogel particles dispersed in the elastomeric matrix, wherein the blade applicator is positioned in a trailing position with respect to a surface and

20

wherein the functional material diffuses from the elastomeric matrix to the surface.

2. The applicator according to claim 1, wherein the elastomeric matrix comprises a material selected from the group consisting of polysiloxane, polyurethane, polyester, polyfluorosiloxanes, polyolefin, fluoroelastomer, synthetic rubber, natural rubber, and mixtures thereof.

3. The applicator according to claim 1, wherein the functional material is selected from the group consisting of 10 alkanes, fluoroalkanes, alkyl silanes, fluoroalkyl silanes alkoxy silanes, siloxanes, glycols or polyglycols, mineral oil, synthetic oil, natural oil, and mixtures thereof.

4. The applicator according to claim 1, wherein the functional material comprises a paraffin oil.

5. The applicator according to claim 1, wherein a weight ratio of the functional material to the elastomeric matrix is from about 1 to 10 to about 1 to 2.

6. The lubricant applicator according to claim 1, wherein the elastomeric matrix comprises pores having a size of from 20 about 10 nm to about 100 μm.

7. The applicator according to claim 1, further comprising a mechanism to fix and press the blade applicator against the surface.

8. The applicator according to claim 1, wherein a geometry 25 of a tip the blade applicator is selected from a group consisted of a polygonal prism, triangular prism, a cuboid, and a sphere.

9. The applicator according to claim 1, wherein the blade applicator comprises a thickness of from about 0.1 mm to about 50 mm.

10. The applicator according to claim 1, wherein blade applicator further comprises a outer layer comprising a elastomeric material having pores smaller than pores in the elastomeric matrix to control diffusion of the functional material on the surface.

11. An image forming apparatus comprising:

a) an imaging member having a charge retentive surface for developing an electrostatic latent image thereon, wherein the imaging member comprises:

a substrate, and

a photoconductive member disposed on the substrate;

b) a charging unit for applying an electrostatic charge on the imaging member to a predetermined electric potential; and

c) an applicator disposed in contact with the surface of the imaging member or a surface of the charging unit, wherein the applicator comprises:

a blade applicator comprising an elastomeric matrix and a functional material dispersed therein, wherein the blade applicator is positioned in contact and in a trailing position with respect to the surface of the imaging member or the surface of the charging unit, wherein the functional material comprises paraffin oil and the elastomeric matrix comprises a cross-linked polydimethylsiloxane (PDMS).

12. The image forming apparatus according to claim 11, further comprising a mechanism to fix and press applicator blade against the surface of the imaging member or the surface of the charging unit.

13. The image forming apparatus according to claim 11, 60 wherein a weight ratio of the functional material to the elastomeric matrix is from about 1 to 10 to about 1 to 2.

14. An applicator for use in an image forming apparatus comprising:

a blade applicator comprising a first layer comprising an elastomeric matrix and a functional material dispersed therein, and a second layer comprising an elastomeric material having pores smaller than pores in the elasto-

meric matrix, the second layer disposed on the first layer wherein the second layer is positioned in a trailing position with respect to a surface and wherein the functional material diffuses through the second layer to the surface, wherein the second layer controls diffusion of the functional material to the surface. 5

15. The applicator according to claim 14, wherein the first layer comprises a thickness of from about 1 mm to about 30 mm and pores having a size of from about 1 micron to about 50 microns. 10

16. The applicator according to claim 14, wherein the second layer comprises a thickness of from about 0.01  $\mu\text{m}$  to about 5 mm. 15

17. The applicator according to claim 14, further comprising aerogel particles dispersed in the elastomeric matrix of the first layer. 15

18. The applicator according to claim 14, wherein the functional material comprises paraffin oil.

\* \* \* \* \*